

No. 33,949.

PATENTED DEC. 17, 1861.

M. LANE.  
PROCESS OF MAKING IRON AND STEEL.



Witnesses:

*James D. Dickey*  
Deputy C. Lawrence  
W. S. Cobb

*Marcus Lane*  
Inventor  
of the  
Robt. W. Lawrence  
Attorneys

# UNITED STATES PATENT OFFICE.

MARCUS LANE, OF WASHINGTON, DISTRICT OF COLUMBIA.

## IMPROVEMENT IN PROCESSES OF MAKING IRON AND STEEL.

Specification forming part of Letters Patent No. 33,949, dated December 17, 1861.

*To all whom it may concern:*

Be it known that I, MARCUS LANE, of the city of Washington, in the District of Columbia, have invented a new and Improved Mode of Treating Metals, of which the following is a specification.

The nature of my invention consists in the proper decarbonization and purification of metal while the same is in the act of rotary motion in a concave-bottomed refining-chamber of a refining-furnace auxiliary and adjacent to the stack-furnace in which the metal is fused. I am aware, however, that the mere production of rotary motion in fused metal is neither new nor patentable, and I am also aware that air has been used to produce such motion and decarbonize the metal. But, having discovered new and, as I believe, superior agents for producing such motion and decarbonization, I will proceed to describe their application and use in such manner that any person skilled in the art may be enabled to use and practice my invention, reference being had to the accompanying drawings, forming a part of this my specification, in which—

Figure 1 is a front elevation of an ordinary stack-furnace, its hearth communicating with a refining-furnace, within which, in a refining-chamber, motion to the metal is imparted and the decarbonization takes place. Fig. 2 is a horizontal section of the same, and clearly shows the connection between the hearth of the "stack" and the refining-chamber of the refining-furnace. Fig. 3 is a vertical longitudinal view of the refining-furnace, and shows the connection of the refining-chamber with the chimney of the stack-furnace. Fig. 4 is a vertical longitudinal section of the carbon and alkali reservoirs and a portion of the pipe upon which they are seated.

In the several figures the same letters are used to indicate like or analogous parts.

A indicates the stack-furnace, into which tuyere-pipes b are introduced, as shown, to convey blasts of air to the mass of ore in the stack for the purpose of fusing the same. These tuyere-pipes are connected with apparatus for generating the blasts in any of the well-known modes.

c is the tymp-hole in front of the hearth of the stack-furnace, through which the fused metal is flowed into the gutter d, and thence into refining-chamber e of the refining-fur-

nace F, previous to the refining process in said refining-chamber.

G is a small furnace situated beneath the refining-chamber, having doors h h for the introduction of fuel, and an ash-pit, i, beneath. The rear of furnace G connects with the chimney of the stack-furnace A by means of a flue, j, the flue j entering said chimney at a point near the entrance of the same by the tuyere-pipes b, and against or opposite the mass of ore upon the grate of the stack-furnace.

K is a door or damper giving admission into the refining-chamber e through opening l, for the removal of the slag which accumulates upon the top of the fused metal in the refining-chamber, and which damper, during the refining or decarbonizing process, is closed, so that the blasts introduced into the refining-chamber, as hereinafter described, together with the gases which accumulate in said chamber, will be forced out passage m into flue j, and thence be passed into contact with the ore in the stack-furnace.

N, Fig. 4, indicates a cup-shaped reservoir, having an air-tight cover fitted thereon, as shown. The interior p of this reservoir connects with channel q of the pipe upon which the reservoir is seated. Connection between the reservoir and the pipe is effected by turning cock r, which, at will, may be made to form a communication between the interior of the reservoir and the pipe below it. Two such reservoirs are represented in Fig. 3, one marked N and the other N', the former of which is used to contain alkali and the latter to contain carbon, as hereinafter described.

Previous to drawing the fused metal from the stack-furnace a fire is kindled in furnace G, beneath the refining-chamber e, in order to take the chill from the metal produced by exposure to the air during its transfer from the stack-furnace to the refining-chamber, as well as the chill which otherwise would be produced by the contact of the fused metal with the cold surface of the refining-chamber. The metal in a fluid state is introduced into chamber e of the refining-furnace by running the same from the hearth of the stack-furnace A through the gutter d. The gutter d, being placed tangential to the wall of the refining-chamber e, the metal is caused by its gravitating impetus to assume a rotary motion within the chamber e by reason of its contact with

the sides and concave bottom of said chamber. Such motion having been thus obtained, a blast of steam is thereupon introduced into the chamber *e* through pipe *s*, which is so arranged in its entrance into the chamber as to cause such motion to be continued by its blast. At the same time, in order to prevent the too sudden decarbonization of the metal, carbon—as, for example, charcoal—is introduced from the chamber *N'* through the pipe *s'* by means of a blast of air or steam. The carbon thus introduced comes in contact with the metal at its surface, and is infused throughout the mass, as hereinafter described. Simultaneously with the introduction of the carbon, stop-cock *r* is opened and a quantity of alkali, previously placed in the chamber *N*, is carried by the force of the blast in the pipe *s* into the molten metal.

The mode of introducing the alkali and the carbon is as follows: The alkali, in a powdered state, is placed in the chamber *N*, Figs. 2 and 3, and carbon in a like state is placed in chamber *N'*, same figures. The stop-cocks then, upon being opened, permit the entrance of the alkali and carbon into the pipes *s* and *s'*, and the blasts passing through said pipes convey the alkali and carbon into chamber *e*. By these means I contemplate a double process to be simultaneously carried on in the act of refining metal, and to be applied while the molten metal is in rotary motion in the refining-chamber *e*—to wit, the application of the alkalies operating to effect the formation of slag, and the consequent separation of those earthy impurities in the metal which are not converted into gases by the application of the carbon, and the carbon operating to carry off in the shape of gases those impurities in the metal, which, but for its application, would still remain notwithstanding the formation of the slag by the application of the alkalies. To illustrate: The effect of introducing an alkali—say the carbonate of soda—is as follows, to wit. This alkali is decomposed by the intense heat into carbonic oxide and sodium. The carbonic oxide unites with the carbon in the metal to promote combustion, while the sodium unites with the silicon of the metal, for which it has a greater affinity than has the iron. The union therefore of the silicon and sodium, when oxidized, forms a slag, the nature of which may be described as impure glass, and which may be removed at the pleasure of the operator through opening *l* of the refining-chamber. The effect of introducing carbon is as follows: The oxygen of the air or steam introduced with it forms a carbonic oxide, which unites with the phosphorus and sulphur present in the metal, and for which the carbonic oxide has a strong affinity. The intense heat, acting upon and facilitating the union of the carbonic oxide with said impurities, effects the conversion of them into impure gas, which, being lighter than the air, ascend through passage *m* in the top of the refining-chamber into flue *j*, and thence

into and through the stack. These impure gases pass off by flue *j* in an inflamed state, and in said flue are met by the products of combustion passing off from the furnace *G* below the refining-chamber, and commingling with such products, are together, in an inflamed state, forced into the stack through the terminus of said flue *j*, at such point as to act as an auxiliary tuyere, and be utilized for the fusing of the ores in the stack-furnace.

One advantage of using steam for the infusion of alkali and the production of motion in the molten metal is owing to the fact that a pressure can be obtained upon the molten mass to keep it in motion, of at least two hundred pounds to the square inch, whereas under the use of air for a like purpose a pressure of only some fourteen pounds to the square inch can practically be obtained. Such use of steam, therefore, enables me to treat a much larger mass of metal in a given time than has heretofore been done. Another reason why the use of steam is preferable for giving motion to the metal in the refining-chamber may be stated as follows: Air when introduced is separated by the intense heat of the molten mass into its elements, oxygen and nitrogen. Of these oxygen alone is of use in refining or otherwise changing the nature of the metal, because the nitrogen exists in a negative form or condition, having, so far as can be discovered, no power for the formation of gases by combining with the impurities of the metal; nor has it, so far as can be discovered, any power to assist in the fusing of the ores in the stack-furnace as has the other gases which rise from the chamber *e* through flue *j* into the stack-furnace such, for example, as are formed by the combination of the carbonic oxide with the phosphorus and sulphur, the process of the formation of which is elsewhere described. Steam by being introduced into the molten metal is likewise decomposed into its original elements—namely, oxygen and hydrogen. The oxygen has the same effect and performs the same functions as the oxygen of the air when air is used; and the hydrogen, instead of existing in a negative state, as does the nitrogen, not only combines with the oxygen and the carbon to increase the heat, but also unites with the impurities of the metal to form gases, which, in an inflammable state, pass through the flue *j* into the stack-furnace and materially contribute to the fusion of the ores in said stack-furnace.

I would here state that I do not deem it new, neither do I intend to broadly claim the introduction of carbon to metal at a point above its surface while it is in a fused state; but I do deem it new to introduce carbon to fused metal at a point above its surface while such metal is in rotary motion; and I deem the benefit of such introduction to be this: That the carbon is drawn into the vortex or eddy produced by the rotation, and, sinking with the metal to the bottom of the refining-chamber, is by the subsequent motion of the metal diffused

through its whole mass, the motion of rotation being such by the means I employ as to cause the metal at the bottom to pass to the sides of the refining-chamber, thence up the sides of said chamber to the surface, and thence down again to the bottom of the refining-chamber, the horizontal rotary motion, the ascent, and the descent of the metal creating the vortex or eddy into which the carbon is injected, and so in the first instance brought in contact with the surface of the metal, and by the repeated movements of the metal, as above described, finally permeated throughout its whole mass.

When in the operation of refining metal, as above described, by the simultaneous use of the agents employed, the impurities in the metal have been converted into slag, and have also been passed off in the condition of impure gases, the chambers N and N' are closed, and the blasts applied through the pipes s and s' being continued causes the immediate decarbonization of the metal.

Having thus described my said invention, what I claim as new, and desire to secure by Letters Patent of the United States, is—

1. The simultaneous application of agents other than decarbonizing agents for the purpose of refining and carbonizing metals which act simultaneously not only to carry off the

impurities in the metal in the condition of gases, but also the impurities of the metal in the condition of slag.

2. The simultaneous use of a carbonizing and decarbonizing agent in treating fused metals, which shall act to delay the final decarbonization of the metal to a time at which the impurities shall have been removed by the agents employed.

3. The introduction of carbon at a point above the surface of a mass of fused metal while the metal is in rotary motion.

4. The introduction of the gases from a refining-furnace into the stack of a smelting-furnace in such position and in an inflamed state as to assist in fusing the ore by being passed into the smelting-furnace in immediate contact with the ore.

5. Causing the gases evolved from the fused metal, and which have accumulated in the refining-chamber, to be forced into and among the fusing metal in the smelting-furnace:

6. The introduction of carbonate of soda and the alkalies at a point below the surface of the fused metal in a refining-chamber while the metal is in rotary motion.

MARCUS LANE.

Witnesses:

GUSTAVUS DIETREICH,  
DEWITT C. LAURENCE.